# EUROPEAN PATENT SPECIFICATION

(11) **EP 2 620 486 B1**
(45) Date of publication and mention of the grant of the patent: **24.12.2014**
(21) Application number: 11826874.7
(22) Date of filing: 21.09.2011
(51) Int. Cl.: C10L 1/32, C10L 1/12

(54) **WATER-MIXED FUEL AND METHOD FOR PRODUCING SAME**
MIT WASSER GEMISCHTER KRAFTSTOFF UND HERSTELLUNGSVERFAHREN DAFÜR
COMBUSTIBLE MÉLANGÉ AVEC DE L'EAU ET SON PROCÉDÉ DE PRODUCTION

(30) Priority: 24.09.2010 JP 2010213072
(43) Date of publication of application: 31.07.2013
(73) Proprietor: Marinex Corporation, Nagasaki 857-0852 (JP)
(72) Inventor: FUKUDA, Toshiro, Sasebo-shi Nagasaki 857-0851 (JP); SHIGEMATSU, Toshinobu, Sasebo-shi Nagasaki 857-1193 (JP); SHIMADA, Hideki, Sasebo-shi Nagasaki 857-1193 (JP)
(74) Representative: Winter, Brandl, Fürniss, Hübner, Röss, Kaiser, Polte - Partnerschaft mbB
(86) International application number: PCT/JP2011/071503
(87) International publication number: WO 2012/039429

(56) References cited:
- JP-A- S5 343 706
- JP-A- S58 213 091
- JP-A- S62 106 992
- JP-A- S62 167 391
- JP-A- 2007 125 475
- JP-A- 2009 126 874
- JP-B2- H0 633 373
- JP-B2- S5 824 478
- US-A1- 2009 000 186

## Description

The present invention relates to a water-mixed fuel in which a fuel oil and water are mixed, and a method for producing the same.

### BACKGROUND ART

It is conventionally known that the mixing of water into fuel can reduce engine output. Burning of water is, on the other hand, studied. For example, Non-patent Document 1 discloses an engine capable of providing thermal energy by allowing water and magnesium to react. In addition, an emulsion fuel produced by adding water and a surfactant to a fuel oil is also developed (see, for example, Patent Documents 1 to 3).

### PRIOR ART DOCUMENTS

### PATENT DOCUMENTS

Patent Document 1: Japanese Patent Laid-open Publication No. 2001-348579
Patent Document 2: Japanese Patent Laid-open Publication No. 2000-263062
Patent Document 3: Japanese Patent Laid-open Publication No. 6-346071

### NON-PATENT DOCUMENT

Non-Patent Document 1: "Tenkenkun no Omosiro Shin Gijutsu 4 "MAGIC ENGINE" - a circulating clean energy system", SEIBI in Tokyo, July 2006, [online], TOSSNET, [searched on September 15, 2010], Internet <URL: http://tossnet.or.jp/staticContents/public_html/mtou_tokyoweb/gallery/2006/omosiro20 0607.pdf>

US 2009/0000186 A1 discloses nano-sized metal and metal oxide particles for more complete fuel combustion. Especially is disclosed a fuel composition comprising a liquid fuel and from about 0.01 ppm to about 500 ppm of one or more nano-sized metal or metal oxide particles selected out of a large number of metals and metal oxides. At least 90% of the particles have a size from about 1 to about 990 nm.

### SUMMARY OF THE INVENTION

### PROBLEMS TO BE SOLVED BY THE INVENTION

An object of the present invention is to provide a water-mixed fuel in which a fuel oil and water are mixed through a completely different approach from the above-mentioned conventional methods, and a method for producing the same.

### SOLUTIONS TO THE PROBLEMS

The water-mixed fuel oil for a diesel engine according to the present invention comprises a light oil, 0.2 to 1.0 wt% of water, and 0.02 to 0.06 wt% of a titanium oxide powder as a metal oxide powder, wherein the titanium oxide powder has a particle size of 10 µm or less.

The method for producing a water-mixed fuel oil for a diesel engine according to the present invention comprises the step of mixing a light oil, 0.2 to 1.0 wt% of water, and 0.02 to 0.06 wt% of a titanium oxide powder as a metal oxide powder, wherein the titanium oxide powder has a particle size of 10 µm or less.

According to the present invention titanium oxide is used as the metal oxide powder.

The metal oxide powder has a particle size of 10 µm or less. The particle size of 10 µm or less allows the water and the metal oxide in the water-mixed fuel to be sufficiently in contact with each other, so that the metal oxide powder can function as a catalyst with high efficiency. Such particle size can further prevent the metal oxide powder from damaging the inside of an engine which burns the water-mixed fuel. The particle size of more than 10 µm may deteriorate the function of the catalyst.

### EFFECTS OF THE INVENTION

(1) With the water-mixed fuel containing a fuel oil, water, and a metal oxide powder, the metal oxide powder serves as a catalyst.
(2) As the metal oxide powder has a particle size of 10 µm or less, the water and the metal oxide in the water-mixed fuel are sufficiently in contact with each other, so that the metal oxide powder can function as a catalyst with high efficiency, which in turn improves combustion efficiency. Such particle size can further prevent the powder from damaging the inside of a motor which bums the water-mixed fuel.

### BRIEF DESCRIPTION OF THE DRAWINGS

FIG. 1 is a graph showing experimental results obtained in the case where water in the water-mixed fuel is set from 0.04 to 1.00 wt%, and titanium oxide powder is set to 0.02 wt%, 0.04 wt%, and 0.06%.
FIG. 2 is a graph showing experimental results obtained in the case where water in the water-mixed fuel is set from 0.04 to 1.00 wt%, and titanium oxide powder is set to 0.08 wt%, 0.10 wt%, and 0.12%.
FIG. 3 is a graph showing experimental results obtained in the case where water in the water-mixed fuel is set from 0.04 to 1.00 wt%, and titanium oxide powder is set to 0.14 wt%, 0.16 wt%, and 0.18%.

### EMBODIMENTS OF THE INVENTION

The water-mixed fuel according to an embodiment of the present invention is produced by mixing a fuel oil, water, and titanium oxide powder as a metal oxide powder. Light oil is used as the fuel oil. As the metal oxide powder, powder having a particle size of 10 µm or less obtained by grinding titanium oxide in a mortar or the like is used. Water in the water-mixed fuel is set to 0.2 to 1.0 wt%, and the metal oxide is set to 0.02 to 0.06 wt%.

When the water-mixed fuel is used as a fuel oil for a diesel engine, the titanium oxide powder serves as a catalyst. Further, the titanium oxide powder has a particle size of 10 µm or less, so that it may not damage the inside of the engine.

### EXAMPLES

A measurement test for engine efficiency was conducted with the water-mixed fuel according to an embodiment of the present invention. The water-mixed fuel in this Example was produced by the following process: water was supplied in a specified amount to 1 liter of light oil, the mixed fluid was stirred with a stirrer, titanium oxide as a metal oxide was ground in a mortar to a powder, the powdered metal oxide was further supplied in a specified amount to the stirred fluid, and the mixture was then stirred. In Comparative Example, a water-mixed fuel in which water but no titanium oxide was mixed was used.

The engine efficiency was determined by measuring the acceleration of an actual vehicle. $F = m ⁢ \frac{{d}^{2} . x}{d ⁢ {t}^{2}}$

Referring to the equation above, the acceleration is in proportion to the engine output. m is not merely a mass but a synthesized mass including output efficiency and friction of the engine. Therefore, the measurement of the acceleration also means that the amount proportional to the engine output has been measured. It should be noted that the measured value is not an absolute value but a relative value.

The measuring method follows the procedures below.
(1) Supply a fuel into a diesel engine of an actual vehicle.
(2) Measure the acceleration under conditions of full depression of an accelerator pedal in first gear.
(3) Drain the fuel.
(4) Supply an additive-free light oil into the engine and warm the engine.
(5) Drain the fuel.
(6) Change the conditions of the water-mixed fuel and repeat the steps (1) to (5).

The experimental results are shown in FIGS. 1 to 3. FIG. 1 is a graph showing experimental results obtained in the case where water in the water-mixed fuel is set from 0.04 to 1.00 wt%, and titanium oxide powder is set to 0.02 wt%, 0.04 wt%, and 0.06%; FIG. 2 is a graph showing experimental results obtained in the case where water in the water-mixed fuel is set from 0.04 to 1.00 wt%, and titanium oxide powder is set to 0.08 wt%, 0.10 wt%, and 0.12%; and FIG. 3 is a graph showing experimental results obtained in the case where water in the water-mixed fuel is set from 0.04 to 1.00 wt%, and titanium oxide powder is set to 0.14 wt%, 0.16 wt%, and 0.18%. As a Comparative Example, experimental results of a water-mixed fuel in which water alone is mixed are shown in FIGS. 1 to 3.

As shown in FIG. 1, in the case of the titanium oxide powder of 0.02 to 0.06 wt%, the acceleration of the water-mixed fuel of the Example in the range from 0.2 to 1.00 wt% of water was approximately higher than that of the water-mixed fuel of the Comparative Example in which water alone was mixed, so that it was possible to confirm the improvement of the engine output. As shown in FIG. 2, in the case of the titanium oxide powder of 0.08 to 0.12 wt%, the acceleration of the water-mixed fuel of the Example was higher than that of the water-mixed fuel of the Comparative Example in which water alone is mixed, so that the improvement of the engine output was expected. Depending on the water content, however, the engine output was reduced below that of the Comparative Example in some cases.

As shown in FIG. 3, in the case of the titanium oxide powder of 0.14 wt%, it was confirmed that depending on the water content, the acceleration of the water-mixed fuel of the Example was higher than that of the water-mixed fuel of the Comparative Example in which water alone was mixed. In the case of the titanium oxide powder of 0.16 wt% and 0.18 wt%, however, the acceleration of the water-mixed fuel of the Example was less than that of the water-mixed fuel of the Comparative Example, so that the improvement of the engine output was not confirmed.

### INDUSTRIAL APPLICABILITY

The water-mixed fuel and the method for producing the same according to the present invention are useful as a fuel oil for a diesel engine and as a method for producing the fuel oil.

## Claims

1. A water-mixed fuel oil for a diesel engine comprising a light oil, 0.2 to 1.0 wt% of water, and 0.02 to 0.06 wt% of a titanium oxide powder, wherein the titanium oxide powder has a particle size of 10 µm or less.

2. A method for producing a water-mixed fuel oil for a diesel engine comprising the step of mixing a light oil, 0.2 to 1.0 wt% of water, and 0.02 to 0.06 wt% of a titanium oxide powder, wherein the titanium oxide powder has a particle size of 10 µm or less.

## Patentansprüche

1. Mit Wasser gemischtes Kraftstofföl für einen Dieselmotor umfassend ein Leichtöl, 0,2 bis 1,0 Gew.-% an Wasser und 0,02 bis 0,06 Gew.-% eines Titanoxid-pulvers, wobei das Titanoxidpulver eine Teilchengröße von 10 µm oder weniger aufweist.

2. Verfahren zur Herstellung eines mit Wasser gemischten Kraftstofföls für einen Dieselmotor umfassend den Schritt des Mischens eines Leichtöls, 0,2 bis 1,0 Gew.-% an Wasser und 0,02 bis 0,06 Gew.-% eines Titanoxidpulvers, wobei das Titanoxidpulver eine Teilchengröße von 10 µm oder weniger aufweist.

## Revendications

1. Fioul mélangé à l'eau destiné à un moteur diesel comprenant une huile légère, 0,2 à 1,0 % en poids d'eau, et 0,02 à 0,06 % en poids d'une poudre d'oxyde de titane, dans lequel la poudre d'oxyde de titane a une taille de particule de 10 µm ou moins.

2. Procédé de production d'un fioul mélangé à l'eau destiné à un moteur diesel comprenant l'étape de mélange d'une huile légère, de 0,2 à 1,0 % en poids d'eau, et de 0,02 à 0,06 % en poids d'une poudre d'oxyde de titane, dans lequel la poudre d'oxyde de titane a une taille de particule de 10 µm ou moins.
